

# UNITED STATES PATENT OFFICE.

FELIX KUNERT AND EDWIN ACKER, OF OFFENBACH-ON-THE-MAIN, GERMANY,  
ASSIGNORS, BY MESNE ASSIGNMENTS, TO THE CHEMICAL FOUNDATION, INC.,  
A CORPORATION OF DELAWARE.

## MULTICOLOR PRINTING.

1,426,299.

Specification of Letters Patent. Patented Aug. 15, 1922.

No Drawing.

Application filed November 2, 1916. Serial No. 129,115.

To all whom it may concern:

Be it known that we, FELIX KUNERT and EDWIN ACKER, subjects of the German Emperor, residing at Offenbach-on-the-Main, 5 Germany, have invented new and useful Improvements in Multicolor Printing (for which we have filed applications in Germany, Ser. No. 25,990, filed Feb. 12, 1916, No. 26,036, filed March 1, 1916; Holland, 10 Ser. No. 7,049, filed June 23, 1916), of which the following is a specification.

Hitherto it has not been possible to use nitrosamine colours in multi-colour printing simultaneously with other dyestuffs, such as 15 tannin dyestuffs or chrome dyestuffs, or with steam black, because the nitrosamine colours, that is to say mixtures of nitrosamines and naphthols, cannot stand even a short steaming, since such treatment either causes them 20 to lose strength and fade, or changes their tint; red, for instance, changing towards brown.

The present invention is based on the discovery that nitrosamine colours, to which 25 have been added normal chromates or other metal salts, such as aluminium borate or sodium vanadate, which form with azo-dye- 30 stuffs lakes capable of resisting steam, are satisfactorily fast to steam, so that by using such nitrosamine printing colours the dye- 35 stuff can be developed in tints of full strength and purity after steaming.

Such nitrosamine colours as contain normal chromates or the aforesaid salts may be 40 steamed together with other colours, simultaneously printed, in the Mather-Platt or other steaming apparatus, without exhibiting the aforesaid objection. This was not possible in the processes hitherto known.

Naphthols suitable for use in this invention are all oxynaphthalenes which are capable of acting as components of azo-dyestuffs, and, therefore, in addition to the naphthols themselves derivatives of them, such as arylides of oxynaphthoic acids, or hydrazides of these acids, aminonaphthols, acidyl-aminonaphthols or like bodies may be employed.

In specifications Nos. 199143 and 205461 45 processes are described for reserving indigo by means of nitrosamine-β-naphthol colours with the aid of chromates. These are cases in which normal alkali chromate is added in addition to other chromates to nitrosamine 50 colours but merely for the purpose of reserv-

ing indigo, for a steaming process does not come into question.

The said specifications, therefore, in describing the use of normal chromates for the purpose of reserving indigo do not lead to 60 the deduction that by using nitrosamine colours to which normal chromates have been added, it is possible to develop the dyestuffs satisfactorily after steaming.

The present invention is an important 65 technical advance for it provides many new combinations in printing and renders it possible to print simultaneously with tannin dye- 70 stuffs and chrome dyestuffs, or sulphurized dyestuffs and vat dyestuffs with nitrosamine colours, which was not possible hitherto.

The invention may be carried out by printing on white goods the colours prescribed in the following examples, drying, hanging and steaming for 5-10 minutes in the Mather- 75 Platt apparatus and then developing in a boiling bath containing acetic acid and Glau- 80 ber's salt, or in a bath containing acetic acid and a bichromate, to which in the case of tannin dyestuffs an antimony salt is also added.

A modification of the invention consists in using the nitrosamine printing colours, so far as they contain chromate, in the indigo colour discharge. In this case beautiful and 85 fast discharge effects are obtained on goods dyed with indigo, when the nitrosamine colours are steamed after the printing, and thus for the first time it is possible to use nitrosamine colours for multi-colour dis- 90 charge effects on indigo, because, for instance, in addition to discharge white and nitrosamine-red, yellow or other pigment colours, with albumin and chromate or other steam dyestuffs, can be produced. 95

### A. Nitrosamine colours.

#### EXAMPLE 1.

15 grams β-naphthol.

15 grams caustic soda lye of 34° Baumé 100 specific gravity.

100 grams water.

500 grams tragacanth thickening 1:20.

100 grams nitrosamine of paranitraniline (containing 14 per cent of base). 105

30 grams normal potassium chromate.

240 grams water.

1 kilo.

An orange-red is obtained.

110

## EXAMPLE 2.

- 20 grams  $\beta$ -naphthol.  
 20 grams caustic soda lye of 34° Baumé specific gravity.  
 5 100 grams water.  
 500 grams tragacanth thickening 1:20.  
 110 grams nitrosamine of para-nitro-ortho-anisidine (containing 17 per cent of base).  
 10 50 grams normal sodium chromate.  
 200 grams water.

1 kilo.  
 A blue-red is obtained.

## EXAMPLE 3.

- 15 grams 2:3-oxynaphthoic acid anilide.  
 22 grams caustic soda lye of 34° Baumé specific gravity.  
 20 500 grams tragacanth thickening 1:20.  
 60 grams nitrosamine of meta-nitro-para-toluidine (containing 16 per cent of base).  
 50 grams normal potassium chromate.  
 25 353 grams water.

1 kilo.  
 A turkey-red is obtained.

## EXAMPLE 4.

- 30 20 grams di-2:3-oxynaphthoyl-para-phenylenediamine.  
 30 grams caustic soda lye of 34° Baumé specific gravity.  
 35 500 grams tragacanth thickening 1:20.  
 50 grams nitrosamine of dianisidine (containing 20 per cent of base).  
 370 grams water.  
 30 grams iron chromate (liquid).  
 40 20 grams normal potassium chromate.

1 kilo.  
 A black-blue is obtained.

## EXAMPLE 5.

- 45 20 grams benzoyl-1:7-aminonaphthol.  
 25 grams caustic soda lye of 34° Baumé specific gravity.  
 500 grams tragacanth thickening 1:20.  
 50 75 grams nitrosamine of meta-nitro-para-toluidine (containing 16 per cent of base).  
 340 grams water.  
 40 grams normal potassium chromate.

55 1 kilo.  
 A brownish red is obtained.

## B. Auxiliary colours.

- 20 grams chrome printing yellow 2 G N.  
 60 280 grams water.  
 600 grams starch tragacanth thickening.  
 100 grams chromium acetate of 20° Baumé specific gravity.

65 1 kilo.

- 10 grams methylene blue G.  
 50 grams lactic acid.  
 5 grams tartaric acid.  
 275 grams water.  
 600 grams starch tragacanth thickening. 70  
 60 grams tannin-acetic acid 1:1.

1 kilo.

## C. Developing bath.

- 30 grams acetic acid of 8° Baumé specific 75 gravity.  
 50 grams Glauber's salt, crystallized.  
 20 grams antimony fluoride double salt made up to 1 litre.  
 Application of the process on an indigo 80 ground: On goods dyed with indigo blue is printed:

## (a) Nitrosamine colours.

1. 20 grams  $\beta$ -naphthol. 85  
 20 ccm. caustic soda lye of 34° Baumé specific gravity.  
 100 ccm. water.  
 500 grams thickening.  
 120 grams nitrosamine of para-nitro-ortho-anisidine (containing 17 per cent of base).  
 150 grams normal potassium chromate.  
 90 90 ccm. water.
2. 22 grams 2:3-oxynaphthoic acid anilide. 95  
 20 ccm. caustic soda lye of 34° Baumé specific gravity.  
 208 ccm. water.  
 500 grams thickening.  
 100 100 grams nitrosamine of meta-nitro-para-toluidine (containing 15 per cent of base).  
 150 grams normal potassium chromate.

## (b) Auxiliary colours. 105

- 400 grams Grela yellow R as paste.  
 225 grams tragacanth thickening 1:20.  
 120 grams sodium bichromate.  
 20 ccm. ammonia.  
 35 ccm. water.  
 200 grams egg albumin in water 1:1.

After drying, the goods are steamed for 3-5 minutes in the Mather-Platt apparatus and then passed during 10 seconds through 115 a hot discharge bath consisting of 50 grams oxalic acid and 200 ccm. hydrochloric acid of 20° Baumé specific gravity in 1 litre, and finally well washed.

We claim as our invention:

1. The process of multi-color printing with mixtures of nitrosamines and naphthols upon white goods, comprising printing on said goods with nitrosamine printing colors to which have been added metallic 125 salts which form color lakes uninfluenced by steaming and subsequently developing in a bath containing an organic acid having two atoms of carbon in its molecule.
2. The process of multi-color printing 130

- with mixtures of nitrosamines and naphthols upon white goods, comprising printing on said goods with nitrosamine printing colors to which have been added metallic salts, which form color lakes uninfluenced by steaming, drying, steaming for several minutes, and finally developing in a hot bath containing acetic acid, and a metallic salt. 5
- 10 3. The process of multi-color printing with mixtures of nitrosamines and naphthols upon white goods, comprising printing on said goods with nitrosamine printing colors to which have been added normal chromates, which form color lakes uninfluenced by steaming, drying, steaming about five to ten minutes, and finally developing in a hot bath containing acetic acid and a metallic salt. 15
- 15 4. The process of multi-color printing with mixtures of nitrosamines and naphthols upon white goods, comprising printing on said goods with a nitrosamine printing color
- composed of a derivative of an oxynaphthoic acid, caustic alkali, a thickening agent, 25 a nitrosamine color, water and an aluminium compound, drying, steaming for several minutes, and finally developing in a hot bath containing acetic acid, and a metallic salt. 30
5. The process of multi-color printing with mixtures of nitrosamines and naphthols upon white goods, which comprises printing on said goods with a nitrosamine printing color composed of 2.3 oxynaphthoic acid, caustic soda of 34° Bé. strength, 35 tragacanth thickening, nitrosamine of para-nitraniline, water, and an aluminium compound, drying, steaming for about five to ten minutes, and finally developing in a hot bath containing acetic acid and a metallic salt. 40

Frankfort-o-M. this 8th day of July  
1916.

FELIX KUNERT.  
EDWIN ACKER.